



the following test in which oils to which the inhibitor has been added were subjected to conditions which are more severe than those encountered in the actual operation of internal combustion engines.

Weighed cadmium-silver alloy bearings were submerged in samples of a highly refined oil with and without the addition of the compound to be tested and the oil air agitated while maintained at a temperature of about 341° F. At regular intervals the cadmium-silver alloy bearings were removed from the bath, washed free of oil, and weighed to determine the loss in weight. The bearings were then replaced in the oil and further tested. The oil used was a motor oil refined to such an extent that a loss in weight of more than 5 mg/cm.<sup>2</sup> is obtained in 25 hours or less on a cadmium-silver alloy bearing submerged in the air agitated oil at about 340° F., 20 which oil has been preoxidized for 25 to 50 hours at about 340° F.

The following results were obtained on cadmium-silver alloy bearings when tested in the foregoing manner.

| Oil                                 | Duration of test                      |         |          |
|-------------------------------------|---------------------------------------|---------|----------|
|                                     | 25 hrs.                               | 50 hrs. | 100 hrs. |
|                                     | Loss in weight (mg/cm. <sup>2</sup> ) |         |          |
| Control                             | 2.5                                   | 35.0    | 105.0    |
| Control + 2% mercapto-benzothiazole | 0.0                                   | 0.0     | 0.4      |

The above data definitely show the high inhibiting effect of the mercapto benzothiazole.

Although I prefer to use the compounds of the hereinabove type which are completely oil soluble, equally effective results are obtained with those which are not completely soluble in the lubricant by suspending the inhibitor in the lubricant by means of a small amount of a peptizing agent, such as aluminum naphthenate, 45 aluminum stearate and the like.

While I have described my invention by using preferred examples thereof I do not wish to be limited by the same except as defined by the appended claims.

50 I claim:

1. The method of preventing corrosion of bearing metal alloys selected from the group consisting of cadmium-silver alloys, cadmium-nickel alloys and copper-lead alloys in the presence of

highly refined lubricating oils normally corrosive to said bearing metal alloys in internal combustion engines which comprises adding to said lubricating oils a mercapto benzothiazole in a small but sufficient quantity to effect the retardation of said corrosion to said bearing metal alloys.

2. The method of preventing corrosion of hard metal alloy bearings in the presence of highly refined lubricating oils normally corrosive to said hard metal alloy bearings in internal combustion engines which comprises adding to said lubricating oils a bivalent radical substituted five-membered ring compound having sulfur and nitrogen in the ring and having the general formula



in which X is a radical selected from the group consisting of a benzo radical and an arylene derivative of a benzo radical, R is a substituent selected from the group consisting of hydrogen, an alkyl radical, an aryl radical and R<sub>1</sub> is a substituent selected from the group consisting of hydrogen, an alkyl radical, an aryl radical, an amino group and a mercapto group, said compound being added to said lubricating oil in a small but sufficient quantity to effectively inhibit the corrosion to said hard metal alloy bearings.

3. The method of preventing corrosion of hard metal alloy bearings in the presence of highly refined lubricating oils normally corrosive to said hard metal alloy bearings in internal combustion engines which comprises adding to said lubricating oils a benzothiazole having the general formula



in which R is a substituent selected from the group consisting of hydrogen, an alkyl radical and an aryl radical, and R<sub>1</sub> is a substituent selected from the group consisting of hydrogen, an alkyl radical, an aryl radical, a mercapto group and an amino group, said benzothiazole being added to said lubricating oil in a small but sufficient quantity to effectively inhibit the corrosion of said hard metal alloy bearings.

CLARENCE M. LOANE.